# EUROPEAN PATENT SPECIFICATION

(11) **EP 0 007 233 B1**
(45) Date of publication and mention of the grant of the patent: **28.04.1982**
(21) Application number: 79301377.2
(22) Date of filing: 12.07.1979
(51) Int. Cl.: C25D 11/16, B41N 3/00, C25F 3/04

(54) **A method of treating aluminium foil or a lithographic printing plate support and products so obtained**
Verfahren zur Behandlung von Aluminiumfolien oder Flachdruckplatten sowie die so erhaltenen Produkte
Procédé de traitement de feuilles d'aluminium on de plaques lithographiques et produits obtenus de cette mainère

(30) Priority: 13.07.1978 GB 2970578
(43) Date of publication of application: 23.01.1980
(73) Proprietor: BICC Public Limited Company, London, WC1B 3QN (GB)
(72) Inventor: Thomas, Alan, Windle, St. Helens Merseyside (GB); Rowlands, David Philip, Sale, Cheshire M33 5PU (GB)
(74) Representative: Poole, Michael John

## Description

This invention relates to the treatment of aluminium (including its alloys); especially aluminium foil in continuous web form. Primarily, but not exclusively, it is concerned with the pre-treatment of aluminium that is subsequently to be coated with photosensitive material to make a presensitised lithographic printing plate.

Aluminium for this purpose is almost always anodised, generally using a bath based on sulphuric acid, though phosphoric acid is used by at least one manufacturer. Sulphuric acid gives a hard, adherent and abrasion-resistant coating, but there are problems in getting satisfactory adhesion of some attractive sensitive coatings (for example polyvinyl cinnamate among negative-working coatings and orthoquinone diazide sulphonate-based resists amongst positive-working coatings). Phosphoric acid anodising gives much better adhesion with these and some other coatings, but the anodic coating is much softer and tends to abrade away during printing to an extent that may limit the number of copies that can be taken off the plate.

In some cases aluminium that has been anodised in sulphuric acid has been treated subsequently with phosphoric acid, and this has been found to give a useful improvement in adhesion while retaining part of the advantages of the use of sulphuric acid for anodising, but this presents obvious difficulties in control of the operation.

DE-A 2557222 illustrates the use of an auxiliary electrolytic cell as a mere means for introducing current into a web of aluminium foil for the purpose of anodising it, and US-A 3929591 describes a process in which, prior to being anodised, an aluminium foil is etched in an entirely separate A.C. anodising process.

The invention is based in part on the realisation that anodic oxidation takes place at the surface of the metal, not of the coating, and that it will not of itself destroy the existing exposed surface of the coating.

In accordance with the invention, a method of treating aluminium comprising passing the web through a first bath containing phosphate ions and afterwards through an anodising bath containing sulphate ions is characterised by passing current between an anode immersed in the first bath and a cathode immersed in the anodising bath.

The web may be passed through the baths by dipping or, with some advantages, by spraying or flooding the surface of the aluminium.

The phosphate ions are preferably orthophosphate ions, but more complex phosphates can be used.

The phosphate and sulphate ions may be the only anions present to any substantial extent in the respective baths, but the presence of other anions that are inert or that modify, rather than radically alter, the effect of the treatment may be present. In particular the presence of minor amounts of sulphate in the phosphate bath and/or of phosphate in the sulphate bath is not excluded. We prefer that the associated cations should be wholly or mainly hydrogen ions, but neutral or alkaline salt solutions may be suitable in some cases.

### Example

The accompanying drawing shows the distinctive part of apparatus in which a web of aluminium foil 1 is passed, on the run, through a first bath 2 containing 45% aqueous orthophosphoric acid and, with or without intermediate washing (not shown), through a second bath 3 containing 15% sulphuric acid. Current is supplied from a conventional power pack and flows between an inert anode 4 immersed in the first bath and an inert cathode 5 immersed in the second bath via both the electrolytes and the part 6 to the aluminium web extending between the two baths. Under typical conditions the bath temperatures are both around 20°C, the applied potential is about 16.5 V and the mean current density at each of the immersed length of the foil is about 200 Am-2. The line speed is such that the dwell time in each bath is approximately four minutes.

After washing and drying the anodised web is coated with a proprietary positive-working lithographic resist comprising a resin sensitised with the 2,4 dihydroxybenzophenone ester of 1, 2, 5 diazo naphthol sulphonic acid and coloured with a blue dye to yield presensitised plates with excellent adhesion and press life compared with the best current commercial anodised- aluminium presensitised lithographic printing plates. The anodic coating is thin compared with conventional coatings, and penetration of dye into the coating is not significant.

## Claims

1. A method of treating aluminium foil in web form comprising passing the web through a first bath containing phosphate ions and afterwards through an anodising bath containing sulphate ions characterised by passing current between an anode immersed in the first bath and a cathode immersed in the anodising bath.

2. A method of making a presensitised lithographic printing plate comprising anodising aluminium sheet or foil and subsequently applying a lithographic photosensitive coating to it, characterised in that the sheet or foil is treated by the method claimed in Claim 1.

3. Aluminium foil treated by the method claimed in Claim 1.

4. A presensitised lithographic or printing plate made by the method claimed in Claim 2.

## Revendications

1. Procédé de traitement de l'aluminium en feuille sous forme de bande consistant à faire passer cette bande dans un premier bain contenant des ions phosphate, caractérisé en ce qu'on fait passer un courant entre une anode immergée dans la premier bain et une cathode immergée dans la bain d'anodisation.

2. Procédé pour fabriquer une plaque d'impression lithographique présensibilisée comprenant l'anodisation d'une tôle ou feuille d'aluminium et ensuite l'application d'un revêtement lithographique photosensible sur cette feuille, ce procédé étant caractérisé en ce qu la tôle ou feuille est traitée par le procédé suivant la revendication 1.

3. Aluminium en feuille, caractérisé en ce qu'il est traité par le procédé suivant la revendication 1.

4. Plaque d'impression ou lithographique présensibilisée, caractérisée en ce qu'elle est fabriquée par lé procédé suivant la revendication 2.

## Patentansprüche

1. Verfahren zur Behandlung von Aluminiumfolien in Form einer Bahn, die durch ein erstes, Phosphationen enthaltendes Bad geführt wird, dadurch gekennzeichnet, daß zwischen einer in das erste Bad eingetauchten Anode und einer in ein anodisch oxidierendes Bad eingetauchten Kathode ein Strom fließt.

2. Verfahren zum Herstellen einer vorsensibilisierten lithographischen Druckplatte durch anodisches Oxidieren eines Bleches oder einer Folie aus Aluminium und anschließendes Aufbringen einer lithographischen, photoempfindlichen Beschichtung, dadurch gekennzeichnet, daß das Blech oder die Folie durch das Verfahren nach Anspruch 1 behandelt wird.

3. Aluminiumfolie, behandelt durch das Verfahren nach Anspruch 1.

4. Vorsensibilisierte Lithographie- oder Druckplatte hergestellt durch das Verfahren nach Anspruch 2.
